

G. S. YINGLING.  
MEDICATED INSOLE FOR FOOTWEAR.  
APPLICATION FILED MAR. 18, 1914.

1,113,726.

Patented Oct. 13, 1914.

*Fig. 1.*



*Fig. 2.*

Witnesses

Fenton H. Bell  
J. M. Sherwood

Inventor  
George S. Yingling  
By Franklin H. Douglass  
H. H. [Signature]  
Attorney

# UNITED STATES PATENT OFFICE.

GEORGE S. YINGLING, OF EAU GALLIE, FLORIDA,

## MEDICATED INSOLE FOR FOOTWEAR.

1,113,726.

Specification of Letters Patent. Patented Oct. 13, 1914.

Application filed March 18, 1914. Serial No. 825,600.

To all whom it may concern:

Be it known that I, GEORGE S. YINGLING, a citizen of the United States, residing at Eau Gallie, in the county of Brevard and State of Florida, have invented certain new and useful Improvements in Medicated Insoles for Footwear; and I do hereby declare the following to be a full, clear, and exact description of the invention, such as will enable others skilled in the art to which it appertains to make and use the same, reference being had to the accompanying drawings, and to the letters and figures of reference marked thereon, which form a part of this specification.

This invention relates to new and useful improvements in insoles for shoes, footwear, etc., and comprises a simple and efficient device of this nature, made preferably of the matted fiber of the palmetto tree which has been suitably treated with tannic acid.

I have illustrated in the drawing forming a part of this application views of insoles made of palmetto and in which:

Figure 1 is a plan view of a sole, and Fig. 2 is an enlarged detail view of a portion of one of the soles showing the manner of the intersecting hairlike fibers of the palmetto.

In treating, the fiber A, before being made up into insoles, having a circumferential binding B of cloth stitched thereto, or other purpose for which it is to be used, is sprayed or otherwise treated with a mixture of coal oil (kerosene) and oil of myrbane, preferably in the proportions of one gallon of coal oil to one ounce of myrbane. This mixture as it acts upon the fiber which naturally contains a considerable amount of tannic acid, incorporated within the fiber, will in no way interfere with the elasticity of the fiber or its usefulness as an insole or as a filler for mattresses or other purposes for which it may be employed. After the treatment of

the insole with the mixture of oil of myrbane and coal oil, the palmetto fiber remains 45 impregnated therewith without affecting the tannic acid which exists in the fiber, the tannic acid serving to repel insects by reason of its bitterness as well as serving to preserve the fiber in a similar manner as 50 would be the effect of the tannic acid upon tanning hides in the manufacture of leather.

By the provision of insoles made of the palmetto fiber, when treated in the manner described, I have found that the burning 55 and sweating of feet will be prevented, a soft means to cushion the feet will be afforded and any impurities which may be given off through the pores of the feet will be absorbed by the fiber, the feet being kept 60 cool in hot weather and warm in cold weather. The fiber, which is of light texture and elastic, will be airy and a non-conductor of heat and cold and will produce a perfectly healthy insole, capable of being 65 washed and dried repeatedly without in any way injuring the fiber.

The palmetto fiber treated in accordance with my method will insure the same against any insects, such as red bugs, jiggers, fleas, 70 etc., and will impart an agreeable fragrance to the foot and shoe of the wearer.

What I claim to be new is:

An insole for shoes and other footwear made up of a matted fiber of the bark of 75 the palmetto tree, containing tannic acid in its makeup, and impregnated with a mixture of coal oil and oil of myrbane, as set forth.

In testimony whereof I hereunto affix my 80 signature in presence of two witnesses.

GEORGE S. YINGLING.

Witnesses:

LILA PERSONS,  
JNO. E. M. HODGSON.